# EUROPEAN PATENT SPECIFICATION

(11) **EP 0 540 991 B1**
(45) Date of publication and mention of the grant of the patent: **15.04.1998**
(21) Application number: 92118367.9
(22) Date of filing: 28.10.1992
(51) Int. Cl.: B41M 5/00

(54) **Thermal transfer recording image receiving sheet**
Bildempfangsschicht für thermische Farbstoffübertragung
Feuille réceptrice d'images pour l'enregistrement par transfert thermique

(30) Priority: 05.11.1991 JP 288721/91
(43) Date of publication of application: 12.05.1993
(73) Proprietor: KONICA CORPORATION, Tokyo 163 (JP)
(72) Inventor: Takeyama, Toshihisa, Konica Corporation, Hino-shi, Tokyo (JP); Kitamura, Shigehiro, Konica Corporation, Hino-shi, Tokyo (JP); Koshizuka, Kunihiro, Konica Corporation, Hino-shi, Tokyo (JP)
(74) Representative: Türk, Gille, Hrabal, Leifert

(56) References cited:
- EP-A- 0 410 724
- DATABASE WPIL,n 90-086334,Derwent Publications Ltd,London,GB; & JP-A-2038089 (OJI PAPER) 07.02.1990

## Description

### FIELD OF THE INVENTION

This invention relates to a thermal transfer recording image receiving sheet and a method for producing it. More specifically, this invention relates to a thermal transfer recording image receiving sheet and a method for producing it, which cause neither uneven images nor curls at the time of image formation and are capable of forming images in a high sensitivity and a high transfer density.

### BACKGROUND OF THE INVENTION

As methods for obtaining colored hard copies, there have so far been studied color recording techniques such as ink jet recording, electrophotography and thermal transfer recording. Of these methods, thermal transfer recording has, not necessarily limited to the case of color recording, advantages that it is easy to handle and maintain, allows downsizing of apparatus and requires less cost.

This thermal transfer recording includes the heat melt transfer method and the thermo-diffusion transfer method; the latter is also called the thermo-sublimation transfer method, because it uses a sublimation-type thermal transfer recording ink sheet having on a support an ink layer containing a sublimation dye which sublimates on heating and transfers, through diffusion, onto a thermal transfer recording image receiving sheet.

This thermo-diffusion transfer method can control the gradation of an image by varying the amount of dye to be transferred correspondingly to the change in the amount of heat energy applied by a thermal head. Accordingly, it has a distinctive advantage that it can easily form multicolor printed images having a continuous change in color shades by performing a superposition-recording using the three primary colors of cyan, magenta and yellow.

With such an advantage, the thermal transfer recording method of thermo-diffusion transfer type has come to be extensively used in making image recording bodies to record gradational color images such as color photographic images.

However, conventional thermal transfer recording image receiving sheets used in this thermal transfer recording method have problems of causing uneven printing owing to surface irregularities or adhesion of foreign matters and yielding a low transfer sensitivity and an insufficient transfer density.

As a measure to solve these problems, use of a support of porous structure is proposed as described in Japanese Pat. O.P.I. Pub. Nos. 112693/1986, 148293/1987, 152793/1987, 1595/1988, 231984/1988, 44781/1989, 47536/1989, 168493/1989, 92592/1990, etc.

Further, methods for laminating a porous intermediate layer between the support and the image receiving layer are proposed as seen in Japanese Pat. O.P.I. Pub. Nos. 270192/1986, 87286/1988, 122593/1988, 145192/1989, 280586/1989, 89690/1990, 241740/1990, 76687/1991, etc. and methods for laminating an intermediate layer having a cushioning function between the support and the image receiving sheet are proposed as seen in Japanese Pat. O.P.I. Pub. Nos. 144394/1986, 258793/1986, 146693/1987, 151393/1987, 5885/1989, 26497/1989, etc.

In these methods, however, the unevenness in images, though fairly reduced, cannot be prevented enough at all times; moreover, a sufficient transfer density and an enough transfer sensitivity cannot be obtained in times; in the case of intermediate layers having a porous structure, curling cannot be prevented enough on occasion for their insufficient heat stability and dimensional stability. Further, when an intermediate layer is formed by a coating method, curling tends to occur in the drying process after coating because of the thermal shrinkage of the coated layer, besides an environmental problem which may be caused by evaporation of solvents.

In order to prevent such disadvantages, there is proposed extrusion lamination of a polyolefine resin on a base made of wood pulp or natural pulp as described in Japanese Pat. O.P.I. Pub. Nos. 263081/1989, 106397/1990, 305688/1990 and U.S. Pat. Nos. 4,774,224, 4,999,335. When paper is used as a base, curling can be prevented, but there occur at times uneven images attributable to the surface waviness of fibers in the paper as well as insufficient transfer sensitivities and transfer densities due to diffusion of heat during recording.

From JP-A 2/38089 a base sheet for a thermosensitive transfer image accepting sheet is known said base sheet comprising a coated paper which is made by coating a synthetic polymer emulsion (on the paper) said base sheet being laminated with a polyolefine resin such as polypropylene having a thickness of 10 to 200 %m said polyolefine (polypropylene) resin comprising a pigment.

### SUMMARY OF THE INVENTION

The present invention is made to improve the above situation.

Accordingly, the object of the present invention is to provide a thermal transfer recording image receiving sheet and a method for producing it, which are capable of forming images free from unevenness, high in sensitivity and transfer density and immune from curling.

The present inventors have found that the above object is attained by laminating a resin composition containing polypropylene as principal component as defined in claim 1 by melt extrusion.

As a result of a further study, the inventors have found that among the above laminating layers comprising polypropylene as principal component, a laminating layer having a specific thickness is more effective, that addition of a specific additive to this laminating layer is much more effective, and that appropriate contrivances on the base composition and laminated position of a subbing layer can produce favorable results.

The present invention has been accomplished on the basis of these findings and provides a thermal transfer recording image receiving sheet as defined in claim 1, preferred embodiments of which are defined in claims 2 to 6 and a method for producing the sheet of the invention as defined in claim 7 to 9.

In the sheet as defined in claim 1 first subbing layer and/or the second subbing layer may contain at least one of the resins of alkyl titanates, titanium-modified water-borne resins, ethylene-vinyl acetate copolymers, acrylic resins, urethane resins, polyester resins or epoxy resins.

In the sheet as defined in claim 1 said laminated polypropylene layer may contain white fine particles. Said white fine particles may be hollow fine particles.

In the sheet as defined in claim 1 on the opposite side of the support to the image receiving layer, the second resin layer may be coated directly or via the third subbing layer.

Said second resin layer may contain polyolefine as a principal component and may have a thickness of 5 to 100 µm.

Said third subbing layer preferably contains, as a principal component, at least one of the resins of alkyl titanates, titanium-modified water-borne resins, ethylene-vinyl acetate copolymers, acrylic resins, urethane resins, polyester resins or epoxy resins.

The support, or the first resin layer of sheet defined in claim 1 may contain polyethylene terephthalate as a principal component.

Fig. 1 is a schematic diagram to show the construction of the invention.

The invention includes, as shown in the schematic diagram of Fig. 1, a thermal transfer recording image receiving sheet of claim 1 having a support formed of a resin or a support composed of a base having a first resin layer on the surface, a 5- to 100-µm thick laminating layer, of which principal component is polypropylene, laminated on said first resin layer directly or via a first subbing layer, and an image receiving layer having a dyeability to a thermo-diffusible dye and laminated on said laminating layer directly or via a second subbing layer.

The embodiment of claim 2 includes the thermal transfer recording image receiving sheet wherein said first subbing layer and/or said second subbing layer comprises, as principal component, at least one of the resins selected from alkyl titanates, titanium-modified water-borne resins, ethylene-vinyl acetate copolymers, acrylic resins, urethane resins, polyester resins and epoxy resins.

The embodiment of claim 3 includes the thermal transfer recording image receiving sheet of claim 1 or 2 wherein said laminating polypropylene layer layer contains white fine particles.

The embodiment of claim 4 includes the thermal transfer recording image receiving sheet of claim 3 wherein said white fine particles are hollow fine particles.

The embodiment of claim 5 includes, as shown in the schematic diagram of Fig. 1, the thermal transfer recording image receiving sheet stated in any of claims 1 to 4 wherein said second resin layer is laminated directly or via a third subbing layer on the surface of said support oppositely with the image receiving, layer.

A further preferred embodiment includes the thermal transfer recording image receiving sheet of claim 5 wherein said second resin layer contains polyolefine as principal component and has a thickness of 5 to 100 µm.

A further preferred embodiment includes the thermal transfer recording image receiving sheet of claim 5 wherein said third subbing layer comprises, as principal component, at least one of the resins selected from alkyl titanates, titanium-modified water-borne resins, ethylene-vinyl acetate copolymers, acrylic resins, urethane resins, polyester resins and epoxy resins.

The embodiment of claim 6 includes the thermal transfer recording image receiving sheet of claim 1 wherein said support formed of a resin or said first resin layer comprises polyethylene terephthalate as principal component.

The the method for producing a thermal transfer recording image receiving sheet of claim 7 comprises the steps of forming a laminating layer by coating a resin composition comprising polypropylene as principal component as defined in claim 1 to a thickness of 5 to 100 µm through melt extrusion on the surface of a support formed of a resin, or on a first resin layer of a support having said first resin layer on one side, directly or after forming a first subbing layer by lamination and/or coating, and then forming an image receiving layer having a dyeability to a thermo-diffusible dye on this laminating layer, directly, or after forming a second subbing layer by coating and/or lamination.

A further embodiment of claim 7 includes the method for producing a thermal transfer recording image receiving sheet of claim 8 wherein said support is formed by providing a second resin layer, through lamination of a resin, directly or via a third subbing layer, on the surface of said support oppositely with the side on which the image receiving layer is to be formed.

A further embodiment of claim 8 includes the method for producing a thermal transfer recording image receiving sheet of claim 9 wherein said second resin layer is formed to a thickness of 5 to 100 µm by use of a composition comprising polyolefine as principal component.

Fig. 1 is a schematic diagram as described above, and the detailed layered structure according to the invention will become apparent from the description to follow.

### DETAILED DESCRIPTION OF THE INVENTION

The thermal transfer recording image receiving sheet and the method for the production thereof according to the invention are hereinafter described in detail.

### (I) Thermal Transfer Recording Image Receiving Sheet of claim 1 and Method for Producing it (Part 1)

### (I-a) Support

A support formed of a resin or a support composed of a base having the first resin layer at least on one side is used as the above support.

Examples of such a resin or those which form such a resin layer include acrylic resins derived from acrylates and methacrylates; polyester type resins such as polyethylene terephthalates, polybutylene terephthalates, polyethylene naphthalates, polycarbonates, polyarylates; polyolefine type resins such as polyvinyl chlorides, polyvinylidene chlorides, polyvinylidene fluorides, polyethylenes, polypropylenes, polystyrenes; polyamide type resins such as nylons, aromatic polyamides; polyether ether ketones; polysulfones, polyether sulfones, polyimides, polyether imides, polyparabanic acids, phenoxy resins, epoxy resins, urethane resins, melamine resins, alkyl resins, phenol resins, fluororesins and silicone resins.

In view of dimensional stability, it is preferable that the support formed of a resin or the first resin layer in the invention be a sheet or film each subjected to drawing and heat setting. Among the resins described above, favorable ones are polyester type resins such as polyethylene terephthalates, polybutylene terephthalates, polyethylene naphthalates, polycarbonates and polyarylates. And polyethylene terephthalates, polybutylene terephthalates and polyethylene naphthalates, particularly, polyethylene terephthalates are preferred in respect of costs and formability into sheets or film. Further, the support formed of a resin or the first resin layer can be properly selected according to uses from those having no micro-voids and those having micro-voids.

Examples of the support having the first resin layer include plastic films or sheets laminated with two or more of such resin layers; and films or sheets of various high-molecular materials, metals, ceramics and papers made of wood pulp, cellulose pulp or sulfite pulp, which are laminated with the above resin layer.

When the support is employed in uses which require transparency, such as transparent originals for an overhead projector and seals to be put on glass, one having a high transparency is preferred. In the case of reflection images, there may be incorporated in a component layer of the support a white pigment, such as titanium oxide, zinc oxide, silica, barium sulfate, magnesium carbonate, calcium carbonate, talc or clay, for enhancing the sharpness of images formed.

The thickness of the support is appropriately selected within a range of usually 20 to 1,000 µm, preferably 50 to 500 µm.

In the invention, for the purposes of preventing curling and improving texture, the second resin layer may be laminated, directly or via a subbing layer described below (hereinafter occasionally referred to as the third subbing layer), on the support oppositely with the image receiving layer.

The composition of this second resin layer may be the same as, or different from, that of the laminating layer provided on the side of the image receiving layer described later.

The resin to form the second resin layer may be any resin as long as it is less in necking-in and good in drawdown property. Examples thereof include olefine type resins such as high density polyethylenes, medium density polyethylenes, low density polyethylenes, polypropylenes, polybutenes, polypentenes, polystyrenes, ethylene-vinyl acetate copolymers; polyester resins such as polyethylene terephthalates; ionomer resins; nylons and polyurethanes.

Among them, polyolefine type resins are preferred. Particularly, high density polyethylenes, medium density polyethylenes, low density polyethylenes, polypropylenes, polybutenes, polypentenes, ethylene-propylene copolymers are preferably used singly or in combination of two or more kinds.

When polyolefine type resins are used, the thickness of the resin layer is properly selected within a range of usually 5 to 100 µm, preferably 10 to 50 µm.

In the resin layer comprising polyolefine as principal component, there may be added an additive usable in the laminating layer formed on the same side as the image receiving layer described later.

The resin layer can be formed on the support in the same manner as the laminating layer and, if necessary, it may be subjected to calendering for a smooth surface or embossing for a matted surface.

### (I-b) Laminating Layer

In the invention, the laminating layer having a specific thickness and comprising polypropylene as principal component as defined in claim 1 is laminated at least on one side of the support. This laminating layer can be formed by melt extrusion (occasionally called the hot-melt extrusion laminating method).

As compared with polyolefine type resins used in the usual lamination, particularly with polyethylene, polypropylene is high in heat resistance and low in thermal conductivity; therefore, it has preferable capabilities of preventing curling and providing sufficient transfer sensitivities and transfer densities.

Further, it is preferable that the melt flow rate (test method: ASTM D1238) of this polypropylene be within a range of 0.5 to 15 g/10 min, especially within a range of 1 to 10 g/10 min. And, as long as its drawdown property is sufficient, it may be either a homopolymer or a copolymer, or may be a mixture of two or more kinds of polypropylenes.

The thickness of the laminating layer according to the invention can be properly selected within a range of 5 to 100 µm, preferably 10 to 50 µm.

When the thickness is less than 5 µm, cushioning characteristics are poor and uneven images become liable to occur; when the thickness is more than 100 µm, the cushioning characteristics are not improved any more, the balance in thickness between the support and the laminating layer gets worse and, moreover, curling may occur at the time of image formation.

Lamination by melt extrusion can be carried out by the usual methods described in Japanese Pat. O.P.I. Pub. Nos. 263081/1989, 271289/1989, 106397/1990, 111586/1990, 305688/1990, 49991/1991, etc.

For the purposes of raising the whiteness and enhancing the heat resistance of said laminating layer as defined in claim 1, it is preferred to add further white fine particles to the composition comprising polypropylene as principal component.

As the white fine particles described above, either inorganic fine particles or organic fine particles can be used as long as these are good in heat stability during lamination.

Examples of the inorganic fine particles include metal oxides such as silica, titanium oxide, aluminium oxide, zinc oxide, magnesium oxide, aluminium borate; metal salts such as calcium carbonate, magnesium carbonate, barium sulfate, magnesium sulfate, aluminium hydroxide, boron nitride; and kaolin, clay, talc, zinc white, white lead, quartz, diatomaceous silica, pearlite, bentonite, mica and synthetic mica.

Examples of the organic fine particles include melamine resin particles, guanamine resin particles, styrene-acryl copolymer resin particles, silicone resin particles and fluororesin particles.

Among these white fine particles, hollow resin fine particles are preferred for their capabilities of raising the transfer sensitivity or transfer density; examples of such hollow fine particles include bridged styrene-acryl hollow resin particles.

When the above white fine particles are added, the content in the laminating layer is properly selected within a range of usually 1 to 30 wt%, preferably 5 to 20 wt%.

The average particle size of these white fine particles is usually 0.01 to 2 µm, preferably 0.02 to 1 µm.

Besides the above white fine particles, the laminating layer may contain additives such as antistatic agents, thermal stabilizer, antioxidants, UV absorbents, light stabilizers and optical whitening agents, which do not decompose at the laminating temperature.

The addition amount of these additives is selected to be usually not more than 30 wt%, preferably not more than 20 wt%.

In the invention, when the adhesion between the support and the laminating layer is not sufficient, it is preferable that the resin layer be subjected to a surface treatment prior to the lamination of a composition comprising polypropylene as principal component on the support.

This surface treatment can be performed by use of the conventional resin surface modification techniques such as the corona discharge treatment, flame treatment, ozone treatment, ultraviolet light treatment, irradiation treatment, roughening treatment, chemical treatment, low temperature plasma treatment and grafting treatment. Details to perform these treatments can be seen in Chapter 2 of "Kobunshi Hyomen No Kiso To Oyo, Ge (Fundamentals and Applications of Polymer Surfaces, Part 2)" by Kagaku Dojin Co., Chapter 8 of "Kobunshi Shinsozai Binran (Handbook of New Polymeric Materials)" by Maruzen Co., etc. These treatments may be carried out in combination of two or more kinds.

The support provided with the laminating layer in the above manner may be subjected to heat setting under the control of dimensions to improve the dimensional stability, or the laminating layer may be subjected to calendering or embossing when necessary.

### (I-c) Image Receiving Layer

In the invention, an image receiving layer is formed on the laminating layer provided as above.

There is no particular restriction on this image receiving layer as long as the layer has a dyeability to a thermo-diffusible dye. According to uses, it can be formed of various materials, with various compositions and in various layer configurations. It may be formed similarly to an image receiving layer comprising a conventional material, composition and layer configuration, or a proper modification may be made on these matters.

Suitable resins for forming such an image receiving layer are, for example, polyvinyl chloride type resins, polyvinylidene chloride type resins, polystyrene type resins, polyester type resins, acrylic resins, epoxy resins, phenoxy resins, polyvinyl acetal type resins, cellulosic resins, polyvinyl pyrrolidones, polycarbonates, polysulfones, polyarylates, polyparabanic acids, polyurethane resins and polyamide resins.

These resins may be used singly or in combination of two or more kinds.

In forming the image receiving layer, the above resins may be cross-linked or hardened by means of irradiation, heat, moisture or catalysts which utilize reactive sites of these resins. In such a case, irradiation-curable monomers such as epoxides and acrylates and cross-linking agents such as isocyanates may be used.

Further, when dyes capable of chelating metal ions (capable of forming chelate dye images) are contained in the ink layer of a thermal transfer recording ink sheet as described later, metal-ion-containing compounds may be used in the image receiving layer if necessary.

Examples of such metal-ion-containing compounds include those exemplified in the specification of U.S. Pat. No. 4,987,049.

These metal-ion-containing compounds are added in an amount of preferably 5 to 60 wt%, especially 10 to 40 wt% of the total amount of the components used to form the image receiving layer.

The image receiving layer may contain, if necessary, additives such as releasants, antioxidants, heat stabilizers, UV absorbents, light stabilizers, fillers, pigments and optical whitening agents. Plasticizers or heat-fusible materials may also be contained as sensitizer.

In the invention, the total addition amount of additives is preferably selected within a range from 0.1 to 30 wt% of the resin to form the image receiving layer.

The thickness of the image receiving layer is within a range of usually 3 to 30 µm, preferably 5 to 20 µm.

The image receiving layer may be a single layer or, if necessary, may have a multi-layered structure consisting of the same or different compositions. Further, the image receiving layer may be formed covering the whole laminating layer, or on its limited portions according to a specific requirement.

The image receiving layer can be formed by the coating method comprising the steps of preparing a coating solution to form the image receiving layer by dispersing or dissolving the necessary components in a solvent, then coating and drying the solution on the surface of a layer composed of a composition comprising polypropylene as principal component, or by the hot-melt extrusion laminating method comprising melt extrusion of a mixture of the components to form the image receiving layer.

Solvents usable in the coating method are, for example, water, alcohols, cellosolves, aromatic hydrocarbons, ketones, esters, ethers and chlorinated solvents.

In carrying out the coating, the conventional coating methods, such as engraved-roll coating, extrusion coating, wire bar coating and roll coating, can be employed.

A proper drying after the coating gives an image receiving layer with a prescribed dry coating thickness. When the adhesion between the image receiving layer and the laminating layer is not sufficient, it is preferable that the laminating layer be subjected to a surface treatment prior to the formation of the image receiving layer. This surface treatment is preferably carried out by use of the above-mentioned method applied onto the support. Preferably, this surface treatment is carried out by the above method which is applied to the support; the procedure of the method can be employed without any modification.

### (I-d) Subbing Layer

In the invention, it is preferable that a subbing layer be each formed between the support and the laminating layer, between the laminating layer and the image receiving layer, and between the support and the second resin layer. For the sake of convenient explanation, the subbing layer formed between the support and the laminating layer is hereinafter occasionally referred to as the first subbing layer, the subbing layer formed between the laminating layer and the image receiving layer is referred to as the second subbing layer, and the subbing layer formed between the support and the second resin layer is referred to as the third subbing layer.

These subbing layer can be formed of at least one of resins selected from alkyl titanates, titanium-modified water-borne resins, ethylene-vinylacetate copolymers, acrylic resins, urethane resins, polyester resins and epoxy resins.

The thickness of the subbing layer is properly selected within a range of usually 0.01 to 10 µm, preferably 0.1 to 5 µm.

The subbing layer can be formed by the coating method comprising the steps of dissolving its components in a solvent and coating and drying the solution so-prepared, or by hot-melt extrusion lamination of the components.

Solvents usable in the coating method are conventional solvents such as water, alcohols, methyl ethyl ketone, toluene, dioxane and cyclohexanone.

When the lamination method is employed, co-extrusion with the first resin layer onto the base can also be carried out. Further, an overcoat layer may be laminated, for the purpose of preventing fusing between the thermal transfer recording ink sheet and the thermal transfer recording image receiving sheet.

The thicknes the second resin layer is in a range of usually 5 to 100 µm, preferably 10 to 50 µm and especially 15 to 40 µm.

Further, an overcoat layer may be laminated on the surface of the image receiving layer, for the purpose of preventing fusing between a thermal transfer recording ink sheet and a thermal transfer recording image receiving sheet.

### (II) Thermal Transfer Recording Ink Sheet and Method for Manufacturing It

The thermal transfer recording ink sheet can be formed basically by laminating an ink layer on a support.

### (II-a) Support

The material for the support is not particularly limited as long as it has a sufficient dimensional stability and a stability to the heat applied in recording using a thermal head; examples thereof include tissue paper such as condenser paper, glassine paper; and films of heat resistant plastics such as polyethylene terephthalates, polyethylene naphthalates, polyamides, polyimides, polycarbonates, polysulfones, polyvinyl alcohols, cellophane, polystyrene.

The thickness of the support is preferably 2 to 10 µm.

The form of the support is not particularly limited and may be any of broad films or sheets, narrow tapes and cards.

### (II-b) Ink Layer

The ink layer contains a thermo-diffusible dye and a binder as essential components, when it is used to transfer an image to a thermal transfer recording image receiving sheet by the thermal diffusion transfer method.

Thermo-diffusible dyes include cyan dyes, magenta dyes and yellow dyes. As cyan dyes, the conventional naphthoquinone dyes, anthraquinone dyes and azomethine dyes are used.

Examples of the magenta dyes include the conventional anthraquinone dyes, azo dyes and azomethine dyes.

Examples of the yellow dyes include the conventional methine dyes, azo dyes, quinophthaloin dyes and anthraisothiazole dyes.

Particularly preferred thermo-diffusible dyes are azomethine dyes obtained by coupling of a compound having an open chain or closed chain active methylene group with an oxidation product of a p-phenylenediamine derivative or an oxidation product of a p-aminophenol derivative, and indoaniline dyes obtained by coupling of a phenol or naphthol derivative with an oxidation product of a p-phenylenediamine derivative or an oxidation product of a p-aminophenol derivative.

The thermo-diffusible dye contained in the thermo-diffusible dye containing ink layer may be any of the yellow dye, magenta dye and cyan dye when formation of monochrome images is intended.

To form chelate dye images between a thermo-diffusible dye and a metal ion, a metal-ion-containing compound is incorporated in the image receiving layer, and a dye capable of forming a chelate in conjunction with this metal-ion-containing compound is used as the thermo-diffusible dye.

As a dye capable of forming a chelate in conjunction with a metal-ion-containing compound, a suitable one can be selected from various conventional dyes. Typical examples thereof include the cyan image forming dyes (hereinafter referred to as cyan dyes), the magenta image forming dyes (hereinafter referred to as magenta dyes) and the yellow image forming dyes (hereinafter referred to as yellow dyes) described in Japanese Pat. O.P.I. Pub. Nos. 78893/1984, 109349/1984 and Japanese Pat. Appl. Nos. 213303/1990, 214719/1990, 203742/1990.

Among the above dyes, preferred are those capable of forming at least a two-site chelate in conjunction with the metal-ion-containing. Typical examples of such dyes are those represented by the following formula:

In the formula, X¹ represents a group of atoms necessary to form an aromatic carbocycle or an aromatic heterocycle, in which at least one ring is composed of 5 to 7 atoms and at least one carbon atom adjacent to the carbon atom linked with the azo group is monosubstituted with a nitrogen atom or a chelating group; X² represents an aromatic carbocycle or an aromatic heterocycle, in each of which at least one ring is composed of 5 to 7 atoms; and G represents a chelating agent.

Irrespective of the type of dyes used, there may be contained two or more of the above three types of dyes, or other thermo-diffusible dyes, according to the color tone of an image to be formed.

These thermo-diffusible dyes are used in amounts of usually 5 to 70 wt%, preferably 20 to 60 wt% of the ink layer forming composition.

Suitable binders used in the ink layer are cellulosic resins, polyvinyl acetal type resins, styrene type resins, acrylic type resins, rubber type resins, ionomer resins, olefine type resins, polyester resins, etc.

These binders may be used singly or in combination of two or more kinds.

In addition, the ink layer may properly contain various additives, such as releasing compounds, fillers and curing agents reactive to the binder component (e.g., isocyanates, irradiation-activated compounds including acrylates and epoxides). Moreover, there may also be added heat fusible materials to accelerate the transfer, such as the waxes and higher fatty esters described in Japanese Pat. O.P.I. Pub. No. 106997/1984.

### (II-c) Other Layers

The thermal recording ink sheet is not limited to the double-layered structure comprising the support and the ink layer, and other layers may also be formed.

For example, an overcoat layer may be provided on the surface of the ink layer in order to prevent fusing with a thermal transfer recording image receiving sheet or offsetting of a thermo-diffusible dye. The support may have a subbing layer, for the purposes of improving the adhesion to the binder and preventing transfer or migration of the dye to the support side. Further, a backing layer may be provided on the reverse side of the support (oppositely with the ink layer), in order to prevent the thermal head from fusing or sticking to the support and the thermal transfer recording ink sheet from creasing.

The thickness of the overcoat layer, subbing layer or backing layer is usually 0.1 to 1 µm.

The thermal transfer recording ink sheet can be produced by coating and drying, on the support, a coating solution for ink layer prepared by dispersing or dissolving the above ink layer components.

The above binders are used, singly or in combination of two or more types, after being dissolved or dispersed to a latex-form in a solvent.

Usable solvents are water, ethanol, tetrahydrofuran, methyl ethyl ketone, toluene, xylene, chloroform, dioxane, acetone, cyclohexanone, n-butyl acetate, etc.

The coating of the ink layer can be performed by gravure coating in which the face is coated in sequence, extrusion coating, wire bar coating or roll coating.

The ink layer may be formed as a layer containing monochromatic thermo-diffusible dyes over the whole support surface or on parts of the support surface, or it may be formed in three layers comprising a yellow ink layer, a magenta ink layer and a cyan ink layer arranged on the same plane in a prescribed repetition order, over the whole support surface or on parts of the support surface. Further, a black ink layer containing a black image forming material may be provided in addition to the above three ink layers. Such a black ink layer works in providing a sharp image whether it is used in diffusion transfer or in melt transfer.

The thickness of the ink layer so-prepared is usually 0.2 to 10 µm, preferably 0.3 to 3 µm.

For the sake of convenient handling, the thermal transfer recording ink sheet may have perforations or detection marks to detect the position at which the color changes.

### (III) Image Formation

In forming images, the ink layer of the thermal transfer recording ink sheet is brought into contact with the image receiving layer of the thermal transfer recording image receiving sheet, then heat energy is applied imagewise to the interface of the ink layer and the image receiving layer.

Thereupon the thermo-diffusible dye in the ink layer thermally diffuses or sublimates in an amount corresponding to the amount of heat energy applied at the of this image formation and moves to the image receiving layer side, where it is received to form a dye image (a chelate dye image).

As a heat source to apply the heat energy, a thermal head is usually used. Other conventional ones, such as laser beams, infrared flash lamps and hot pens, can also be employed.

When a thermal head is used as a heat source, the heat energy applied can be changed continuously or stepwise by modulating the voltage or pulse width applied to the thermal head.

When a laser beam is used as a heat source, the amount of the heat energy can be changed by varying the luminous energy or irradiation area of the laser beam.

In this case, it is preferred that a laser beam absorbing material (e.g., carbon black or a near infrared ray absorbing material for a semiconductor laser) be present in or near the ink layer.

In forming images by use of a laser beam, it is preferable that the thermal transfer recording ink sheet be closely contacted with the thermal transfer recording image receiving sheet.

Using a dot generator provided with a built-in acousto-optical element makes it possible to apply the heat energy in an amount corresponding to the size of a dot.

When an infrared flash lamp is used as a heat source, it is preferable that heating be carried out through a colored layer such as black, similarly to the case of laser beams. Heating may also be performed through a pattern continuously expressing shades of an image in black or the like or through a dot pattern. Further, heating may be performed using jointly a colored layer such as a solid black layer and a negative pattern corresponding to a negative of the above pattern.

The heat energy may be applied from the thermal transfer recording ink sheet side, from the thermal transfer recording image receiving sheet side, or from the both sides. But, when priority is given to energy saving, it is preferred to perform heating from the thermal transfer recording ink sheet side.

Through the procedure described above, a monochromatic image is recorded on the image receiving layer of the thermal transfer recording image receiving sheet, and a color image formed by combination of respective colors, like a color photograph, can be obtained according to the following procedure.

For example, when thermal transfer is carried out by exchanging yellow, magenta, cyan and, if necessary, black thermal transfer recording ink sheets one by one, a color image like a color photograph can be obtained in combination of the respective colors. Such a color photograph-like color image can also be obtained using a thermal transfer recording ink sheet having areas coated in respective colors, instead of the above monochromatic thermal transfer recording ink sheets of respective colors. This method has an advantage that the exchange of thermal transfer recording ink sheets is not needed.

After an image is formed as above, a heat treatment may be performed in the above manner in order to improve image preservability. For example, heat is applied all over the image formed area with a thermal head using non-ink portions of an ink sheet, or additional heating with a heat roll may also be performed. Further, when a near infrared ray absorber is contained, the image formed area may be exposed to an infrared flash lamp.

The purpose of the heat treatment is to make the dye diffuse much deeper into the image receiving layer; therefore, it is preferable that the heating be made from the support side of the image receiving layer irrespectively of heating means.

### EXAMPLES

The present invention is hereinafter described in detail with examples, but the invention is by no means limited to these examples. In the examples to follow, the term "parts" means "parts by weight as an active ingredient" unless otherwise specified.

### Examples 1 to 36

### 1. Thermal Transfer Recording Image Receiving Sheets

The thermal transfer recording image receiving sheets shown in Tables 1 and 2 were prepared in the following procedure.

### Supports

a; a 350-µm thick white-pigment-containing white polyvinyl chloride film (Sumilite VSS 3101 made by Sumitomo Bakelite Co.)
b; a 125-µm thick transparent polyethylene terephthalate film (S made by Diafoil Hoechst Co.)
c; a 350-µm thick white-pigment-containing white polyethylene terephthalate film (Melinex made by Imperial Chemical Ind. Ltd.)
d; a 250-µm thick white-pigment-containing white polyethylene terephthalate film (Crisper made by Toyobo Co.)
e; a 100-µm thick white polyethylene terephthalate film (W900J made by Diafoil Hoechst Co.)
f; a support formed by steps of coating and drying the following adhesive layer coating solution on a 50-µm thick white polyethylene terephthalate film (W900J made by Diafoil Hoechst Co.) by wire bar coating to a dry thickness of 2 µm, overlaying the adhesive-layer-coated film so-prepared on both sides of a 60-µm thick woodfree paper base having a smoothness of 250 sec, press-bonding them with a heat roll while taking caution not to entrain bubbles, and heating them for 1 hour at 100°C to cure the adhesive layer, adhesive layer coating solution used:

| | |
|---|---|
| Polyester resin (Vylon 200 made by Toyobo Co.) | 6 parts |
| Curing agent (Coronate HL made by Nippon Polyurethane Ind. Co.) | 4 parts |
| Methyl ethyl ketone | 80 parts |
| Cyclohexanone | 10 parts |

Laminating Compositions (compositions comprising polypropylene as principal component as defined in claim 1)
The following polypropylene compositions were each melted and kneaded thoroughly and then laminated by hot-melt extrusion on the above base in a thickness of 10 to 50 µm to form a laminating layer comprising polypropylene as principal component.
a; a polypropylene having a density of 0.90 g/cm³ and a melt flow rate of 9 g/10 min.
b; a polypropylene containing 5 parts of titanium oxide (average particle size: 0.3 µm) and having a density of 0.90 g/cm³ and a melt flow rate of 9 g/10 min.

c; a polypropylene containing 12 parts of titanium oxide (average particle size: 0.3 µm) and having a density of 0.90 g/cm³ and a melt flow rate of 7 g/10 min.
d; a polypropylene containing 12 parts of cross-linked styrene-acrylate hollow resin particles (average particle size: 0.4 µm, JSR Hollow Particles SX863 (P) made by Japan Synthetic Rubber Co.) and having a density of 0.90 g/cm³ and a melt flow rate of 7 g/10 min.

### Subbing Layers

The following subbing layers were formed on the base (subbing layers classified as A in Table 1), on the laminating layer (subbing layers classified as B in Table 1) and on the base oppositely with the image receiving layer (subbing layers classified as B in Table 1).
a; a subbing layer formed by coating and drying an ethyl acetate solution dissolving 5 parts of alkyl titanate (Orgatix PC-426 made by Matsumoto Kosho Co.) to a thickness of 0.1 µm.
b; a subbing layer formed by coating and drying a 8/32 water/methanol mixed solvent solution dissolving 2.5 parts of a titanium-modified water-borne resin (Orgatix WS680 made by Matsumoto Kosho Co., active component: 11%) to a thickness of 0.1 µm.
c; a subbing layer formed by coating and drying a toluene solution dissolving 10 parts of a composition comprising a ethylene-vinyl acetate copolymer (Adcote AD-1790-15 made by Toyo Morton Co.) as principal component to a thickness of 0.5 µm.
d; a subbing layer formed by coating and drying the following subbing layer coating solution to a thickness of 0.5 µm, and curing the coated layer by heat treatment at 100°C for 1 hour,
the subbing layer coating solution comprised

| | |
|---|---|
| Acryl type resin (Desmophene A450 made by Sumitomo Bayer Urethane Co.) | 7 parts |
| Curing agent (Coronate HL made by Nippon Polyurethane Co.) | 3 parts |
| Methyl ethyl ketone | 80 parts |
| Cyclohexanone | 10 parts |

e; a subbing layer formed as in d to a thickness of 1.0 µm, using a subbing layer coating solution comprising

| | |
|---|---|
| Urethane type resin (made by Takeda Chem Ind., Ltd.Takelac A-367H ) | 7 parts |
| Curing agent (made by Takeda Chem. Ind., Ltd.Takenate A-7 ) | 3 parts |
| Methyl ethyl ketone | 80 parts |
| Cyclohexanone | 10 parts |

f; a subbing layer formed as in d to a thickness of 1.0 µm, using a subbing layer coating solution comprising

| | |
|---|---|
| Polyester type resin (Vylon 103 made by Toyobo Co.) | 7 parts |
| Curing agent (Coronate L made by Nippon Polyurethane Co.) | 3 parts |
| Methyl ethyl ketone | 80 parts |
| Cyclohexanone | 10 parts |

g; a subbing layer formed as in d to a thickness of 1.0 µm, using a subbing layer coating solution comprising

| | |
|---|---|
| Epoxy resin (Epikote 1001 made by Yuka-Shell Epoxy Co.) | 5 parts |
| Curing agent (Epomate B-002 made by Yuka-Shell Epoxy Co.) | 5 parts |
| Methyl ethyl ketone | 80 parts |
| Cyclohexanone | 10 parts |

h; prior to forming a subbing layer, the base surface was subjected to corona discharge.
i; prior to forming a subbing layer, the base surface was irradiated for 10 min with a UV ray (low wavelength type: 189 nm).
j; prior to forming a subbing layer, the base surface was irradiated with an electron beam using a 750-kv electron beam accelerator.
k; prior to forming a subbing layer, the base surface was subjected to a low temperature plasma treatment by being placed in a plasma reaction apparatus of cylindrical flow and polarized external polar type filled with an Ar atmosphere, followed by introduction of acrylonitrile monomers to form a plasma-polymerized thin layer of acrylonitrile on the base surface.

### Image Receiving Layers

The following image receiving layer coating solutions were coated and dried to form image receiving layers having a thickness of 20 µm (a and b) and that of 10 µm (c and d).
a; an image receiving layer coating solution comprising

| | |
|---|---|
| Polyvinyl chloride type resin (vinyl chloride-p-t-butyl benzoate copolymer, Tg: 79°C, polymerization degree: 670, vinyl chloride content: 86.9%) | 6.0 parts |
| Epoxy resin (Epotohto YD-014 made by Tohto Chemical Co.) | 3.5 parts |
| Polyester-modified silicone resin (X-24-8300 made by Shin-Etsu Chemical Co.) | 0.5 part |
| Methyl ethyl ketone | 20 parts |
| Dioxane | 60 parts |
| Cyclohexanone | 10 parts |

b; an image receiving layer coating solution comprising

| | |
|---|---|
| Styrene type resin (Kane Ace B-11A made by Kanegafuchi Chem. Ind. Co.) | 6.0 parts |
| Polyether polyol (Desmophene 550U made by Sumitomo Bayer Urethane Co.) | 2.5 parts |
| Light stabilizer (Irgafos 168 made by Ciba Geigy AG) | 1.0 part |
| Polyester-modified silicone resin (X-24-8300 made by Shin-Etsu Chemical Co.) | 0.5 part |
| Methyl ethyl ketone | 60 parts |
| Dioxane | 20 parts |
| Cyclohexanone | 10 parts |

c; an image receiving layer coating solution comprising

| | |
|---|---|
| Vinyl chloride type resin (vinyl chloride-dimethyl fumarate copolymer, Tg: 74°C, polymerization degree: 620, vinyl chloride content: 83.5%) | 4.5 parts |
| Polyether polyol (Desmophene 550U made by Sumitomo Bayer Urethane Co.) | 2.0 parts |
| Metal-containing compound ([Ni²⁺(NH₂COCH₂NH₂)₃] 2[(C₆H₅)₄B]⁻) | 3.0 parts |
| Polyester-modified silicone resin (X-24-8300 made by Shin-Etsu Chemical Co.) | 0.5 part |
| Methyl ethyl ketone | 60 parts |
| Dioxane | 20 parts |
| Cyclohexanone | 10 parts |

d; an image receiving layer coating solution comprising

| | |
|---|---|
| Styrene type resin (JSR AES110 made by Japan Synthetic Rubber Co.) | 4.0 parts |
| Polyester polyol (Desmophene 670 made by Sumitomo Bayer Urethane Co.) | 2.0 parts |
| Metal-containing compound ([Ni²⁺(NH₂COCH₂NH₂)₃] 2[(C₆H₅)₄B]⁻) | 2.5 parts |
| Zinc oxide (super fine particle zinc oxide Zn-100 made by Sumitomo Cement Co.) | 1.0 part |
| Polyester-modified silicone resin (X-24-8300 made by Shin-Etsu Chemical Co.) | 0.5 part |
| Methyl ethyl ketone | 60 parts |
| Dioxane | 20 parts |
| Cyclohexanone | 10 parts |

Composition Comprising Polyolefine as Principal Component

Each of the following compositions comprising polyolefine as principal component was melted and kneaded sufficiently, then extrusion laminated to a thickness of 10 to 50 µm on a base oppositely with the face on which an image receiving layer to be formed. A layer comprising polyolefine as principal component was thus prepared.
a; a polypropylene having a density of 0.90 g/cm³ and a melt flow rate of 9 g/10 min.
b; a polypropylene containing 5 parts of titanium oxide (average particle size: 0.3 µm) and having a density of 0.90 g/cm³ and a melt flow rate of 9 g/10 min.
c; a polypropylene containing 12 parts of titanium oxide (average particle size: 0.3 µm) and having a density of 0.90 g/cm³ and a melt flow rate of 7 g/10 min.
d; a polypropylene containing 12 parts of cross-linked styrene-acrylate hollow resin particles (average particle size: 0.4 µm, JSR Hollow Particles SX863 (P) made by Japan Synthetic Rubber Co.) and having a density of 0.90 g/cm³ and a melt flow rate of 7 g/10 min.
e; a low density polyethylene having a density of 0.914 g/cm³ and a melt flow rate of 7.0 g/10 min.
f; a low density polyethylene containing 10 parts of titanium oxide (average particle size: 0.3 µm) and having a density of 0.914 g/cm³ and a melt flow rate of 7.0 g/10 min.

### 2. Thermal Transfer Recording Ink Sheets

The ink layer coating solutions shown below were prepared, and each of them was coated by wire coating g on the corona-discharge-treated surface of a 6-µm thick polyethylene terephthalate film (Lumiler F53N made by Toray Ind. Inc.) to a dry coating thickness of 1 µm. On the other side of the film, a nitrocellulose solution containing 50 wt% silicone resin (Dai-Allomer SP-712 made by Dainichiseika Co.) was coated by wire bar coating to a dry coating thickness of 0.3 µm to provide a backcoating layer. Thermal transfer recording ink sheets shown in Tables 1 and 2 were thus prepared.
a; an ink layer coating solution comprising

| | |
|---|---|
| Thermo-diffusible dye (Kayaset Blue 714 made by Nippon Kayaku Co.) | 3.0 parts |
| Polyvinyl butyral (S-Lec BX-1 made by Sekisui Chemical Co.) | 3.0 parts |
| Methyl ethyl ketone | 84 parts |
| Cyclohexanone | 10 parts |

b; an ink layer coating solution comprising

### 3. Formation of Images

An image was formed by steps of bringing the ink layer of the above thermal transfer recording ink sheet and the image receiving layer of the above thermal transfer recording image receiving sheet into contact with each other, and applying the thermal head to the support side of the ink sheet under the conditions described below.

Then, the thermal transfer recording ink sheet was peeled from the thermal transfer recording image receiving sheet, so that an image was recorded on the image receiving sheet.

After the image recording, the printing unevenness, transfer sensitivity, transfer density and curling of the transferred image as well as the adhesion of the image receiving layer were evaluated using the following criteria as shown in Tables 3 and 4.
Lineal density in primary scanning and secondary scanning: 8 dots/mm
Recording power : 0.6 W/dot
Heating time of the thermal head : adjusted stepwise within a range from 20 msec (energy applied: about 11.2∼10⁻³J) to 2 µm sec (energy applied: about 1.12∼10⁻³J)

### Printing Unevenness

The printing unevenness of the transferred image was visually checked.
A: printing unevenness was scarcely observed.
B: printing unevenness was slightly observed.
C: printing unevenness was observed.

### Transfer Sensitivity

The amount of energy applied for giving a reflection density of 1.0 (E) was measured with an optical densitometer for judgement.
A: E ≤ 4.8 × 10⁻³[J]
B: 4.8 × 10⁻³[J]<E ≤ 5.2 × 10⁻³[J]
C: 5.2 × 10⁻³[J]<E ≤ 5.6 × 10⁻³[J]
D: 5.6 × 10⁻³[J]<E

### Transfer Density

The maximum reflection density (OD value) of the image was measured with an optical densitometer.
A: OD value was 2.5 and above.
B: OD value was 2.0 to 2.5.
C: OD value was 1.7 to 2.0.
D: OD value was 1.7 and below.

### Curling

The degree of curling was measured with a curl gauge, its value is expressed as a reciprocal (X) of the radius of curvature given in meters (before recording, the values were all within a range of 0 to 0.5).
A: X<0.5
B: 0.5 ≤ X<1
C: 1 ≤ X<2
D: 2 ≤ X

### Adhesion

Cuts were made in the form of a grid containing 2 mm × 2 mm squares on the image receiving layer side to a depth exceeding the thickness of the polypropylene layer. Then, a tape peeling test was made (Scotch Mending Tape 810 made by Sumitomo 3M Co. was used) to evaluate the adhesive strength.
A: no peeling was observed.
B: only a slight peeling was observed near the cut.
C: less than 20% in number of the squares in the grid were peeled off.
D: more than 20% in number of the squares in the grid were peeled off.

### Comparative Examples 1 to 8

The thermal transfer recording image receiving sheets and the thermal transfer recording ink sheets shown in Table 2, were prepared. After image recording, the printing unevenness, transfer sensitivity, transfer density and curling of the transferred image as well as the adhesion of the image receiving layer were evaluated using the same criteria as those in Examples 1 to 36. The results obtained are shown in Tables 4.

### Supports

g; a 100-µm thick coat paper having a Bekk smoothness of 1500 sec on both sides
   Laminating Composition (composition comprising polypropylene as principal component)
   Instead of the composition comprising polypropylene as principal component, layers having the following compositions were formed.
e; a low density polyethylene having a density of 0.914 g/cm³ and a melt flow rate of 7.0 g/10 min.
f; a low density polyethylene containing 10 parts of titanium oxide (average particle size: 0.3 µm) and having a density of 0.914 g/cm³ and a melt flow rate of 7.0 g/10 min.

**Table 3**

| | Printing Unevenness | Transfer Sensitivity | Transfer Density | Curling | Adhesion |
|---|---|---|---|---|---|
| Comparative Example A | B | B | B | A | C |
| Example 2 | B | B | B | A | C |
| Example 3 | B | B | B | A | C |
| Example 4 | B | B | B | A | B |
| Example 5 | A | B | A | B | B |
| Example 6 | A | B | A | B | B |
| Example 7 | A | B | A | A | B |
| Example 8 | A | B | A | A | B |
| Example 9 | A | B | A | A | B |
| Example 10 | A | B | A | A | B |
| Example 11 | A | B | A | A | B |
| Example 12 | A | B | A | A | B |
| Example 13 | A | B | A | A | B |
| Example 14 | A | A | A | A | B |
| Example 15 | A | A | A | A | B |
| Example 16 | A | A | A | A | B |
| Example 17 | A | A | A | A | B |
| Example 18 | A | A | A | B | B |
| Example 19 | A | A | A | A | B |

**Table 4**

| | Printing Unevenness | Transfer Sensitivity | Transfer Density | Curling | Adhesion |
|---|---|---|---|---|---|
| Example 20 | A | A | A | A | B |
| Example 21 | A | A | A | A | B |
| Example 22 | A | A | A | A | B |
| Example 23 | A | A | A | A | B |
| Example 24 | A | A | A | A | B |
| Example 25 | A | A | A | A | B |
| Example 26 | A | A | A | B | B |
| Example 27 | A | A | A | B | B |
| Example 28 | A | A | A | B | B |
| Example 29 | A | A | A | B | B |
| Example 30 | A | A | A | A | B |
| Example 31 | A | A | A | A | B |
| Example 32 | A | A | A | A | B |
| Example 33 | A | A | A | A | B |
| Example 34 | A | A | A | A | B |
| Example 35 | A | A | A | A | B |
| Example 36 | A | A | A | A | B |
| Comp Example 1 | C | D | D | A | B |
| Comp Example 2 | A | C | B | B | B |
| Comp Example 3 | D | D | D | A | B |
| Comp Example 4 | D | D | D | A | B |
| Comp Example 5 | A | B | C | A | B |
| Comp Example 6 | A | C | C | A | B |
| Comp Example 7 | A | B | C | C | B |
| Comp Example 8 | A | C | C | C | B |

The present invention can provide a thermal transfer recording image receiving layer and a method for the production thereof which are free from printing unevenness, high in sensitivity and transfer density, and immune from curling.

## Claims

1. A thermal transfer recording image receiving sheet comprising:
a resin support or a support having a first resin layer, laminated with a layer comprising a polypropylene homo- or copolymer or a mixture of two or more kinds of polypropylenes as principal component having a thickness of 5 to 100 µm, on the resin support or the first resin layer directly or via a first subbing layer; and an image receiving layer coated on said polypropylene layer directly or via a second subbing layer; and the image receiving layer having a dyability to a thermo-diffusible dye, and which sheet comprises at least the first or the second subbing layer.

2. The sheet of claim 1, wherein at least one of the first subbing layer and the second subbing layer contains at least one compound selected from the group consists of alkyltitanates, titanium-modified hydrophilic resin, ethylene and vinyl acetate copolymers, acrylic resins, urethane resins, polyester resins and epoxy resins.

3. The sheet of claim 2, wherein said polypropylene layer contains a white fine particles.

4. The sheet of claim 3, wherein the white fine particles are a hollow particles.

5. The sheet of claims 1 or 2 to 4, wherein a second resin layer is coated on the support on an opposite side to a side having the image receiving layer, directly or via a third subbing layer.

6. The sheet of claims 1 or 2 to 5, wherein the resin support or the first resin layer contains polyethyleneterephthalate.

7. A method of producing the thermal transfer recording image receiving sheet according to claim 1, wherein, laminating of said polypropylene layer of a thickness of 5 to 100 µm, is made by the melt extrusion method, on the surface of the support or a support composed of a base having a first resin layer on one side, after forming a first subbing layer by coating and/or lamination, and then an image receiving layer having dyeability to a thermo-diffusible dye is laminated on this laminating layer, directly or after forming a second subbing layer by coating and/or laminating.

8. The method of claim 7, wherein the support is formed by providing a second resin layer through lamination of a resin, directly or via a third subbing layer, on one side of the support opposite to the side on which the image receiving layer is formed.

9. The method of claim 8, wherein the second resin layer is formed to a thickness of 5 to 100 µm using a resin of which the principal component is polyolefine.

## Patentansprüche

1. Bildaufnahmefolie für die Thermoübertragungsaufzeichnung, umfassend: einen Harzträger oder einen Träger, der eine erste Harzschicht aufweist, die mit einer Schicht, welche ein Polypropylen-Homo- oder Copolymer oder eine Mischung aus zwei oder mehr Arten von Polypropylenen als Hauptkomponente umfaßt, mit einer Dicke von 5 bis 100 µm auf dem Harzträger oder der ersten Harzschicht direkt oder via eine erste Unterschicht laminiert ist: und eine bildaufnehmende Schicht, die direkt oder via eine zweite Unterschicht auf dieser Polypropylenschicht aufgetragen ist; und wobei die bildaufnehmende Schicht mit einem thermodiffundierbaren Farbstoff färbbar ist und wobei die Folie mindestens die erste oder die zweite Unterschicht umfaßt.

2. Folie nach Anspruch 1, wobei mindestens eine der ersten Unterschicht und der zweiten Unterschicht mindestens eine Verbindung enthält, die ausgewählt wird aus der aus Alkyltitanaten, Titan-modifiziertem hydrophilem Harz, Ethylen- und Vinylacetat-Copolymeren, Acrylharzen, Urethanharzen, Polyesterharzen und Epoxyharzen bestehenden Gruppe.

3. Folie nach Anspruch 2, wobei die Polypropylenschicht feine weiße Partikel enthält.

4. Folie nach Anspruch 3, wobei die feinen weißen Partikel hohle Partikel sind.

5. Folie nach den Ansprüchen 1 oder 2 bis 4, wobei eine zweite Harzschicht auf dem Träger direkt oder via eine dritte Unterschicht auf der entgegengesetzten Seite zu der Seite mit der bildaufnehmenden Schicht aufgetragen ist.

6. Folie nach den Ansprüchen 1 oder 2 bis 5, wobei der Harzträger oder die erste Harzschicht Polyethylenterephthalat enthält.

7. Verfahren zur Herstellung der bildaufnehmenden Folie zur Thermoübertragungsaufzeichnung entsprechend Anspruch 1, wobei das Laminieren der Polypropylenschicht mit einer Dicke von 5 bis 100 µm nach Bilden der ersten Unterschicht durch Auftragen und/oder Laminieren durch die Schmelzextrusionsmethode auf der Oberfläche des Trägers oder eines Trägers durchgeführt wird, der aufgebaut ist auf einer Basis mit einer ersten Harzschicht auf einer Seite, und dann eine bildaufnehmende Schicht mit einer Färbbarkeit durch einen thermodiffundierbaren Farbstoff auf diese laminierende Schicht direkt oder nach Bilden einer zweiten Unterschicht durch Auftragen und/oder Laminieren laminiert wird.

8. Verfahren nach Anspruch 7 - wobei der Träger gebildet wird durch Vorsehen einer zweiten Harzschicht durch Laminieren eines Harzes direkt oder via eine dritte Unterschicht auf einer Seite des Trägers entgegengesetzt zu der Seite, auf der die bildaufnehmende Schicht gebildet wird.

9. Verfahren nach Anspruch 8, wobei die zweite Harzschicht in einer Dicke von 5 bis 100 µm unter Verwendung eines Harzes gebildet wird, dessen Hauptkomponente ein Polyolefin ist.

## Revendications

1. Feuille de réception d'image pour enregistrement par transfert thermique, comprenant:
un support de résine ou un support possédant une première couche de résine, stratifiée avec une couche comprenant un homopolymère ou un copolymère de polypropylène, ou un mélange d'au moins deux sortes de polypropylènes, comme principal composant, avant une épaisseur de 5 à 100 µm, sur le support de résine ou la première couche de résine, directement ou par l'intermédiaire d'une première sous-couche; et une couche de réception d'image déposée sur ladite couche de polypropylène, directement ou par l'intermédiaire d'une deuxième sous-couche; et la couche de réception d'image possédant une capacité de coloration à un colorant thermodiffusible, ladite feuille comprenant au moins la première sous-couche ou la deuxième sous-couche.

2. Feuille selon la revendication 1, dans laquelle au moins une de la première sous-couche ou de la deuxième sous-couche contient au moins un composé choisi dans le groupe constitué par les alkyltitanates, une résilie hydrophile modifiée par du titane, les copolymères d'éthylène et d'acétate de vinyle, les résines acryliques, les résines d'uréthane, les résines de polyester et les résines époxy.

3. Feuille selon la revendication 2, dans laquelle ladite couche de polypropylène contient de fines particules blanches.

4. Feuille selon la revendication 3, dans laquelle les fines particules blanches sont des particules creuses.

5. Feuille selon les revendications 1 ou 2 à 4, dans laquelle une deuxième couche de résine est déposée sur le support sur la face opposée à la face portant la couche de réception d'image, directement ou par l'intermédiaire d'une troisième sous-couche.

6. Feuille selon les revendications 1 ou 2 à 5, dans laquelle le support de résine ou la première couche de résine contient du poly(éthylène-téréphtalate).

7. Procédé de production de la feuille de réception d'image pour enregistrement par transfert thermique selon la revendication 1, dans lequel on effectue la stratification de ladite couche de polypropylène d'épaisseur 5 à 100 µm, par le procédé d'extrusion en fusion, sur la surface du support ou d'un support composé d'une base portant sur une face une première couche de résine, après la formation d'une première sous-couche par enduction et/ou stratification, puis une couche de réception d'image possédant une capacité de coloration à un colorant thermodiffusible est stratifiée sur cette couche de stratification, directement ou après formation d'une deuxième sous-couche par enduction et/ou stratification.

8. Procédé selon la revendication 7, dans lequel le support est formé par placement d'une deuxième couche de résine par stratification d'une résine, directement ou par l'intermédiaire d'une troisième sous-couche, sur une face du support opposée à la face sur laquelle est formée la couche de réception d'image.

9. Procédé selon la revendication 8, dans lequel la deuxième couche de résine est formée sur une épaisseur de 5 à 100 µm avec une résine dont le principal composant est une polyoléfine.
